

## UNITED STATES PATENT OFFICE

2,279,253

## TREATING ALUMINUM SURFACES

Charles J. Slunder, Oakmont, Pa., assignor to  
 Aluminum Company of America, Pittsburgh,  
 Pa., a corporation of Pennsylvania

No Drawing. Application December 23, 1937,  
 Serial No. 181,312

6 Claims. (Cl. 91—68)

This invention relates to the production of oxide-coated aluminum articles having improved surface characteristics, and more particularly to the production of oxide-coated aluminum articles or parts for use in refrigerators and having improved properties.

In the manufacture of various articles of aluminum, it is the practice in some cases to form artificially on the surface thereof a protective coating which is composed substantially of aluminum oxide and generally known in the art as an oxide coating. While aluminum having its surface thus coated has been quite successful commercially, as evidenced by its use in the various arts, for certain applications the inherent properties of the oxide coatings are such that the oxide-coated articles are not wholly satisfactory. For instance, oxide coatings on aluminum surfaces have been found to possess a slight odor, sometimes referred to as a "chalky" or "earthy" odor, which is generally not objectionable and is, in fact, usually unnoticed, but which is sometimes considered undesirable, especially in oxide-coated aluminum articles which in use are normally confined within a relatively small air space, such as articles or parts used in refrigerators.

Another peculiarity of oxide-coated aluminum surfaces is noted when they are used in contact with freezing water, such as the ice-cube trays used in mechanical household refrigerators and the aluminum grids or separators used in them. Considerable difficulty and annoyance have been experienced in removing the ice from oxide-coated aluminum ice-cube trays because of the tendency of the ice formed in contact with an oxide coating to stick or adhere to the surface. This difficulty is overcome to some extent by the provision of levers or other mechanical devices attached to the containers which in use do not reduce the adherence of the ice to the container, but merely afford increased mechanical advantage to permit application of more force in removing the ice. Attempts have also been made to overcome this difficulty by reducing the adherence of the ice to the oxide-coated surface by applying molten wax to the surface of the oxide coating. This solution of the problem is not entirely satisfactory, however, because the covering of the oxide coating with wax and the removal of the excess wax is an operation which adds materially to the cost of production of the article.

It is an object of this invention to provide an article having an oxide-coated aluminum surface which is substantially free of odor. It is

another object of this invention to provide an article having an oxide-coated aluminum surface which has a relatively low adherence to ice formed in contact therewith.

5 It is a primary object of the invention to provide a simple and economical process for the production of oxide-coated aluminum articles such as refrigerator parts, ice-cube trays and the like, which may be substantially free of odor and which present a relatively low adherence to ice formed in contact therewith.

Further objects and advantages of this invention will be apparent from the following description.

15 In the copending application for United States patent, Serial No. 181,311, filed December 23, 1937, by Charles J. Slunder, there is described and claimed a method for the production of oxide-coated aluminum surfaces which are free from the characteristic odor of oxide coatings and have relatively low adherence to ice formed in contact therewith, in which the oxide-coated aluminum surface is treated with an aqueous solution of a sulfuric reaction product.

20 25 The present invention is predicated on the discovery that the effectiveness of a solution of a sulfuric reaction product in reducing the adherence of ice to an oxide-coated aluminum surface can be substantially increased by incorporating in the solution an aqueous wax emulsion. Furthermore, I have found that the sulfuric reaction products act to prevent the breaking of the wax emulsion which ordinarily occurs when plain solutions of such wax emulsions are used in the treatment of oxide-coated aluminum surfaces. Thus, by the method of this invention

30 35 it has been found possible to add the sulfuric reaction product and the wax emulsion to the hot water bath ordinarily used for sealing porous and adsorbent oxide coatings, and to effect the impregnation of the oxide coating with wax and sulfuric reaction product without increasing the number of steps used in the production of ordinary unimpregnated, sealed oxide coatings. The

40 45 50 method of this invention, therefore, permits the production of oxide-coated aluminum surfaces, having very low adherence to ice formed in contact therewith and substantially free from the characteristic odor of oxide-coated aluminum surfaces, in a very economical manner and one which lends itself readily to commercial application.

In the practice of the invention, the aluminum surface is first provided with an adherent and adsorbent oxide coating. The term "oxide coat-

ing" is used herein and in the appended claims to describe a coating consisting substantially of aluminum oxide artificially formed on an aluminum surface by chemical treatment, with or without the use of externally-applied electrical energy, but does not include the thin film of aluminum oxide which is naturally formed on an aluminum surface upon exposure to air. For the purpose of the invention, the oxide coating may be formed on the aluminum surface by any one of several methods, for example, by treating the aluminum article electrolytically as the anode in a solution of sulfuric acid, chromic acid, or oxalic acid, or by treating it, by simple immersion or otherwise, in a hot solution of an alkali carbonate containing a dichromate.

In forming the oxide coating on aluminum refrigerator parts, it is preferred to treat the aluminum surface electrolytically as anode in an aqueous solution of sulfuric acid. The concentration of the acid may range from about 1 to 70 per cent, but I prefer a concentration between 15 and 25 per cent. When a solution containing 15 to 18 per cent of sulfuric acid is used at a temperature of about 68 to 74° F., a current density of about 12 to 13 amperes per square foot is impressed upon the anode, and the action of the electrolyte on the aluminum is allowed to continue for about 10 to 30 minutes.

When using a solution of sodium carbonate and potassium dichromate to produce an oxide coating on an aluminum article, the piece to be coated is preferably immersed in a solution containing about 0.1 to 1.0 per cent of potassium dichromate and 0.5 to 6.0 per cent of sodium carbonate. I prefer to use a solution containing about 2.0 per cent sodium carbonate and 0.5 per cent of potassium dichromate at or near the boiling temperature.

After a suitable oxide coating has been formed on the aluminum surface, it is rendered substantially free from its characteristic odor, and at the same time is provided with the property of low adherence to ice formed in contact with it, by subjecting the oxide coating to the action of an aqueous solution of a sulfuric reaction product containing an emulsified wax in suspension. The sulfuric reaction product may be used in amounts as small as about 0.1 gram per liter and in amounts up to the solubility limit of the compound. For most purposes it has been found desirable to use the sulfuric reaction products in concentrations of 0.5 to 5 grams per liter. The wax used may be any of the water emulsion waxes and is preferably introduced into the solution of the sulfuric reaction product in the form of an aqueous wax emulsion containing about 5 per cent to 30 per cent of wax. The amount of wax emulsion which may be used will vary over a relatively wide range of concentrations, depending on the concentration of the sulfuric reaction product present in the solution. I have found that in order to maintain the emulsified wax in suspension, particularly when the treating solution is to be used hot, it is desirable that the wax be added to the solution of sulfuric reaction product in amounts corresponding to not more than about 5 parts of wax to each part of sulfuric reaction product in solution. In the preferred practice, an aqueous wax emulsion containing about 10 to 25 per cent of wax is used in sufficient quantity to supply 0.25 to 2.5 parts of wax to each part of sulfuric reaction product. The sulfuric reaction product may

be present in amounts in excess of the above proportions up to its solubility limit.

The solution of the sulfuric reaction product containing the wax emulsion may be used at 5 various temperatures, but it is preferred to use it at temperatures above about 80° C. The treatment is carried out preferably by immersing the oxide-coated article in the treating solution at or near boiling for a period of about 30 minutes.

10 The sulfuric reaction products contemplated herein and in the appended claims are the water-soluble inorganic or organic salts of the products produced by the action of sulfuric acid or its equivalent upon aliphatic alcohols of high molecular weight. Compounds of this nature which

have been found to produce satisfactory results are the sulfated or sulfonated fatty alcohols having 12 to 18 carbon atoms, such as lauric, oleic, myristic, cetyl and stearic alcohols, and the like,

20 or mixtures thereof, substantially neutralized with an alkaline medium. These compounds may be formed by methods known in the art by reaction of a fatty alcohol with sulfuric acid or such reagents as fuming sulfuric acid, sulfur trioxide or chlorosulfonic acid, followed by neutralizing

25 the product with an alkali, such as ammonium hydroxide, an alkali metal carbonate or hydroxide, or an organic base such as triethanolamine. According to the conditions of the reaction, either a sulfuric acid ester is obtained by

30 reaction of the hydroxyl group of the alcohol with the sulfuric acid, or aliphatic sulfonic acids, or mixtures of these two types of compounds may be obtained. The use of either or both of these

35 types of compounds is contemplated as falling within the scope of this invention. The water-soluble alkali metal salts of these compounds have been found particularly suitable to the practice of this invention, the sodium salt of the sulfated lauryl, cetyl and stearic alcohols being preferred.

The waxes which have been found suitable for the purposes of this invention are the waxes which may be made to form a substantially stable emulsion with water. Typical examples of such waxes

45 are carnauba wax, paraffin wax, certain types of synthetic waxes, and the like. Any of the usual emulsifying agents may be used, such as alkali metal, ammonium, or ethanolamine soaps, and the like. Aqueous wax emulsions suitable for the purposes of this invention may be formed in various ways known in the art. One emulsion which has been found particularly suitable is an aqueous emulsion of carnauba wax containing about 25 per cent of wax.

50 In the following example there is set forth a comparison of two aluminum ice-cube trays, one of which was treated according to the method of the present invention, the other of which was provided with an aluminum oxide coating and subsequently sealed without the use of the compounds contemplated by this invention. In forming these two trays, they were treated as anodes in a sulfuric acid electrolyte containing 15 per cent sulfuric acid at a current density of about 12 amperes per square foot for a period of about 20 minutes at a temperature of about 70° F. One of the trays was then immersed in a boiling aqueous emulsion prepared by the addition of 5 grams of an aqueous emulsion of carnauba wax containing 25 per cent by weight of wax and 1.35 grams of a sodium salt of sulfated stearic alcohol to each liter of water, for a period of about 20 minutes. The other tray was treated for a like period in boiling water. The trays were then

washed and dried, and it was noted that the characteristic odor of the oxide coating was absent from the tray treated with the wax emulsion and sulfated stearic alcohol composition. Both trays were then filled with water and ice was frozen in them. The trays were then tested by a standard test to determine the pull required to remove the ice from the trays. In this test, it was found that the oxide-coated surface treated with the emulsion required a pull of 65 pounds to remove the ice therefrom, whereas 280 pounds were required for the removal of ice from the tray having the oxide coating which had not been treated with the composition of this invention.

The invention is not to be considered as limited to the coating of refrigerator parts, such as ice-cube trays, grids, and the like, but is adaptable to use in connection with the coating of any aluminum article in which the properties of a substantially odor-free oxide coating and relatively low adherence to ice formed in contact therewith are desired singly or in combination.

The term "aluminum" as used herein and in the appended claims is intended to include both aluminum in its various grades of purity and the aluminum base alloys.

The term "odor-free" as used in this specification and in the appended claims means free from the characteristic odor of oxide coatings.

I claim:

1. An aluminum article provided on its surface with an adherent oxide coating, said coating having been impregnated with an aqueous mixture containing a solution of a material selected from the group consisting of the substantially alkali neutralized sulfonated and sulfated fatty alcohols and the substantially organic base neutralized sulfonated and sulfated fatty alcohols, and a wax emulsion.

2. An oxide-coated aluminum ice-cube tray having a relatively low adherence to ice formed in contact with its surface, said surface comprising an adherent oxide coating, said coating having been impregnated with a mixture containing an aqueous solution of a material selected from

the group consisting of the substantially alkali neutralized sulfonated and sulfated fatty alcohols and the substantially organic base neutralized sulfonated and sulfated fatty alcohols, and a wax emulsion.

3. A method of treating an oxide-coated aluminum surface comprising subjecting said surface to the action of a mixture of an aqueous solution of a material selected from the group consisting of the substantially alkali neutralized sulfonated and sulfated fatty alcohols and the substantially organic base neutralized sulfonated and sulfated fatty alcohols, and a wax emulsion.

4. A method of treating an oxide-coated aluminum surface comprising subjecting said surface to the action of a hot mixture of an aqueous solution of a material selected from the group consisting of the substantially alkali neutralized sulfonated and sulfated fatty alcohols and the substantially organic base neutralized sulfonated and sulfated fatty alcohols, and a wax emulsion.

5. A method of treating an oxide-coated aluminum surface comprising subjecting said surface to the action of an aqueous mixture containing a wax emulsion, and a material selected from the group consisting of the substantially alkali neutralized sulfonated and sulfated fatty alcohols and the substantially organic base neutralized sulfonated and sulfated fatty alcohols in amounts corresponding to not more than about five parts of wax to each part of said substantially neutralized sulfonated and sulfated fatty alcohol.

6. A method of treating an oxide-coated aluminum surface comprising subjecting said surface to the action of an aqueous mixture containing a wax emulsion, and a material selected from the group consisting of the substantially alkali neutralized sulfonated and sulfated fatty alcohols and the substantially organic base neutralized sulfonated and sulfated fatty alcohols in amounts corresponding to about 0.25 to 2.5 parts of wax to each part of said substantially neutralized sulfonated and sulfated fatty alcohol.

CHARLES J. SLUNDER.